

## UNITED STATES PATENT OFFICE.

HARRY A. NOYES, OF GREENWICH, CONNECTICUT, ASSIGNOR TO TEXAS GULF SULPHUR COMPANY, OF BAY CITY, TEXAS, A CORPORATION OF TEXAS.

## SULPHUR-COKE COMPOSITION.

No Drawing.

Application filed August 5, 1924. Serial No. 730,209.

*To all whom it may concern:*

Be it known that I, HARRY A. NOYES, a citizen of the United States, residing at Greenwich, in the county of Fairfield, State 5 of Connecticut, have invented certain new and useful Improvements in Sulphur-Coke Compositions; and I do hereby declare the following to be a full, clear, and exact description of the invention, such as will enable others skilled in the art to which it 10 pertains to make and use the same.

This invention relates to sulphur-coke compositions and has for its object the provision of an improved composition composed for the most part of sulphur and coke.

By sulphur-coke composition I mean a composition composed principally of sulphur and finely divided coke, the coke being distributed substantially uniformly throughout the sulphur in a molten state and the resulting mixture solidified by casting, or otherwise, to form the composition. Such sulphur-coke compositions are useful in the arts and industries for making objects of 20 art, tanks, troughs, tubs, pipes, insulating blocks, and so on, and are of especial advantage where resistance to acid liquors or fumes is desired.

Sulphur compositions composed for the most part of sulphur and finely divided carbonaceous materials, such as coal or graphite, are not in themselves new. I have found, however, that sulphur-coke compositions possess advantageous properties that 30 are not obtainable when coal or graphite are combined in equivalent manner with sulphur. This may be due to the irregular, porous structure of coke. The sulphur-coke composition of my present invention is 40 strong, durable, acid-resistant and can be reliably made of uniform character and properties.

The percentage (by weight) of sulphur in the improved composition of the invention 45 may be varied from about 75% down to about 40%, and, correspondingly, the percentage (by weight) of coke may be varied from about 25% up to about 60%. I prefer, however, to employ from 60 to 45% 50 (by weight) of sulphur and from 40 to 55% (by weight) of coke in making the improved composition of the invention, and my usually preferred composition contains approximately four parts, by weight, of

sulphur to approximately three parts, by 55 weight, of coke. The composition when molten should be fluid enough to pour and flow freely and in this molten state resembles in a general way molten lava.

I have discovered that the size of the coke 60 particles and the relation of the different sized particles to each other have a marked influence upon the ultimate properties of sulphur-coke compositions. Thus, I have found, that a certain composition containing approximately four parts, by weight, of sulphur and three parts, by weight, of coke of a particular and substantially uniform degree of fineness is not strong enough 65 for commercial fabrication and use, and, moreover, loses strength on ageing. If, however, the size of the particles of the coke content of this composition be proportioned in accordance with the principles of my 70 present invention, the resulting sulphur-coke composition is strong, durable and does not deteriorate with age.

I have discovered that the important consideration in making satisfactory compositions of sulphur and coke is to have the 80 proper degrees of fineness of the coke particles, as well as the proper proportions of sulphur and coke. Having established these conditions, i. e., the proper degrees of fineness of the coke particles and the proper 85 proportions of sulphur and coke, additional amounts of finely divided or coarser coke may be added as a filler, or as a reinforcing agent, or for the purpose of giving the composition (in the molten state) the desired 90 consistency for handling or pouring.

The improved composition of the invention in its preferred form, may contain as high as 60 parts of sulphur to 40 parts of coke, by weight, or as low as 45 parts of sulphur 95 to 55 parts of coke. The difference in the relative amounts of sulphur and coke employed in making the composition of the invention depends principally on the amount of coke required to obtain the necessary 100 proportions of coke particles of the proper sizes for body, strength and durability of the product. My usual proportion is approximately four parts of sulphur by weight to three parts of coke by weight. In accordance 105 with the preferred form of the present invention, the coke may conveniently be all finer than 10 mesh (Tyler standard), with

roughly two-thirds of its weight fine enough to pass a 100 mesh screen and from one-half to two-thirds of that which passes the 100 mesh screen fine enough to pass a 200 mesh screen.

The following examples will serve to illustrate the novel features of the invention:-

(1) A sulphur-coke composition made up of about four parts of sulphur and three parts of coke ground to pass a sieve of 200 meshes to the inch was found to have an average initial tensile strength of about 150 pounds per square inch and an average tensile strength of only 28 pounds per square inch after standing for six weeks. On longer standing its tensile strength became substantially negligible.

(2) A sulphur-coke composition made up of around (within 10%) three parts of sulphur and two parts of coke breeze had an initial tensile strength of from 400 to 500 pounds per square inch, but on standing or ageing for a few weeks the tensile strength became substantially lower. The coke breeze employed in this example had the following screen analysis:

|                                            | Per cent. |
|--------------------------------------------|-----------|
| On 10 mesh screen                          | 1.4       |
| 30 Thru 10 mesh screen on 40 mesh screen   | 38.8      |
| 35 Thru 40 mesh screen on 60 mesh screen   | 23.4      |
| 35 Thru 60 mesh screen on 80 mesh screen   | 10.5      |
| 35 Thru 80 mesh screen on 100 mesh screen  | 10.5      |
| 40 Thru 100 mesh screen on 120 mesh screen | 5.0       |
| 40 Thru 120 mesh screen on 150 mesh screen | 2.6       |
| 45 Thru 150 mesh screen on 200 mesh screen | 1.4       |
| 45 Thru 200 mesh screen                    | 6.4       |

(3) A sulphur-coke composition made up as in the preceding example, using for the coke a mixture containing 80% of coke breeze having the foregoing screen analysis and 20% of coke passing a 200 mesh screen, had a tensile strength averaging from 600 to 700 pounds per square inch. Further small changes in the proportions of the particles in the coke mixture gave a composition with a tensile strength of approximately 1000 pounds per square inch.

The sulphur-coke composition of the invention contains by weight from 75 to 40% of sulphur and from 25 to 60% of coke, the coke being of such fineness that from 25 to 75% thereof by weight passes through (and the balance remains on) a 100 mesh screen, and of the part passing through the 100 mesh screen from 40 to 75% thereof by weight passes through (and the balance re-

mains on) a 200 mesh screen. Conveniently, substantially all of the coke is finer than 10 mesh.

As a specific example of the invention, I mention the following composition which I have found to possess excellent properties:

|                                                                         | Pounds.    |
|-------------------------------------------------------------------------|------------|
| Sulphur                                                                 | 60         |
| Coke breeze having approximately the screen analysis hereinbefore given | 76         |
| Coke through 200 mesh                                                   | 28         |
| Coke through 150 mesh on 200 mesh                                       | 10 to 11   |
| Coke through 120 mesh on 150 mesh                                       | 2/3 to 1/3 |
| Coke through 100 mesh on 120 mesh                                       | 2/3 to 1/3 |

Several procedures may be followed in making the sulphur-coke composition of the invention. These procedures will be somewhat dependent upon the size of the container used, the source and amount of heat, the method of mixing, the moisture in the sulphur or coke, and the rapidity with which the moisture is driven off. One procedure is to mix together (dry) the proper materials so that when all or a unit of this mixture is melted, heated, and mixed the proper composition results. Another procedure is to melt the sulphur and to then stir in the coke continuing the heating and stirring after the mixture is complete until the moisture, the occluded air and other gases are driven off. Another procedure is to dry the sulphur and the coke in any convenient manner and then to melt, heat and mix them together. Another method is to heat the coke first and stir the sulphur into the coke with proper heating. Another method is to melt together the whole or a part of the sulphur together with the whole or part of the coke. After the material has solidified, or later, the remaining materials are added and the whole melted, heated and mixed.

After the melting, heating and mixing operation, the molten composition may be cast into the object desired, such as an object of artistic design, a tank, a box, a pipe, an insulating block, and so on, or may be cast into convenient forms (such as sheets, slabs, blocks, etc.) suitable for storage or transportation and until desired for its ultimate use. The molten composition may be sprinkled over a suitable surface, such as a floor, conveyor belt, and the like, where it solidifies in small lumps and fragments resembling frit material. This lump or frit material may be bagged or binned for transportation or storage, as desired.

The temperature of heating in making or recasting the improved composition of the

invention may be just above the melting point of the sulphur or much higher. The advantages of heating to different temperatures depend on the size of the batch, the size of the heater, the purpose for which the material is to be used, the distance it is to be transported in molten state by pipe, pail, etc., the mixing device, and the amount of moisture present in the raw material.

10 The composition is not limited to one casting but may be recast from one shape to another, as desired. This means that it may stay in one cast shape indefinitely or that the same material may comprise the whole 15 or part of several castings or objects inside of a few days, months or years.

From the foregoing description, it will be understood that the present invention contemplates a sulphur-coke composition in 20 which the coke content thereof is of various determined degrees of fineness. Just why it is necessary to have a certain proportion of relatively very fine material and a certain proportion of relatively coarse material 25 with some material in-between these two degrees of fineness, I am not at present prepared to say. As the result of an extended and careful investigation, I have found that these conditions are necessary with respect 30 to the coke content of a satisfactory sulphur-coke composition, and it is my purpose herein to protect this proper sizing of the particles of coke used for the production of superior sulphur and coke compositions that 35 are acid resistant and useful in the arts and industries. It is apparent that I may vary the composition somewhat from time to time on the basis of the difference in area of the surface of the particles making up the 40 proper proportion of coke but carrying the gradation of the particles necessary for the proper composition.

In making the improved sulphur-coke compositions of the invention, I generally 45 use sieved, ground or crushed coke of the proper sizings. I may, if desired, include an appropriate amount of coke breeze, or other available form of finely divided coke, on the basis of its sieve or screen analysis. 50 Petroleum coke (substantially free from iron) and coke screenings (not necessarily all coke) may be included in the total coke content of the composition on the basis of their respective screen analysis.

55 Reinforcing agents, such as expanded metal lath, reinforcing wire or rods, metal screen cloth, etc., may if desired be incorporated or embedded in the sulphur-coke composition, particularly when employed in 60 the construction of tanks and the like where maximum strength is desired.

I claim:—

1. A sulphur-coke composition containing by weight from 75 to 40% of sulphur and 65 from 25 to 60% of coke, the coke being of

such fineness that from 25 to 75% thereof by weight passes through while the balance remains on a 100 mesh screen and of the part through the 100 mesh screen from 40 to 75% thereof by weight passes through while the 70 balance remains on a 200 mesh screen.

2. A sulphur-coke composition containing by weight from 75 to 40% of sulphur and from 25 to 60% of coke, the coke being of such fineness that approximately two-thirds 75 of its weight passes through and the balance remains on a 100 mesh screen and of the part through the 100 mesh screen approximately one-half to two-thirds thereof passes through and the balance remains on 80 a 200 mesh screen.

3. A sulphur-coke composition containing by weight from 75 to 40% of sulphur and from 25 to 60% of coke, the coke being substantially all finer than 10 mesh and from 85 25 to 75% thereof by weight being fine enough to pass through a 100 mesh screen on which the balance remains and of the part through the 100 mesh screen from 40 to 75% thereof by weight being fine enough to pass 90 through a 200 mesh screen on which the balance remains.

4. A sulphur-coke composition containing by weight from 75 to 40% of sulphur and from 25 to 60% of coke, the coke being substantially all finer than 10 mesh with approximately two-thirds of its weight fine enough to pass a 100 mesh screen and approximately one-half to two-thirds of that which passes the 100 mesh screen fine enough 100 to pass a 200 mesh screen.

5. A sulphur-coke composition containing approximately four parts of sulphur by weight and three parts of coke by weight, the coke being substantially all finer than 10 105 mesh with approximately two-thirds of its weight fine enough to pass a 100 mesh screen and approximately one-half to two-thirds of that which passes the 100 mesh screen fine enough to pass a 200 mesh screen. 110

6. A sulphur-coke composition containing approximately four parts of sulphur by weight and three parts of coke by weight, the coke being substantially all finer than 10 mesh and from 25 to 75% thereof by weight being fine enough to pass through a 100 mesh screen on which the balance remains and of the part through the 100 mesh screen from 40 to 75% thereof by weight being fine enough to pass through a 200 115 mesh screen on which the balance remains.

7. A sulphur-coke composition containing by weight from 75 to 40% of sulphur and from 25 to 60% of coke, the coke being made up of approximately 60 to 80% of coke 125 breeze, together with at least 20% of fine coke passing a 200 mesh screen.

8. A sulphur-coke composition containing approximately four parts of sulphur by weight and three parts of coke by weight, 130

approximately two-thirds by weight of the coke being fine enough to pass a 100 mesh screen and approximately one-half to two-thirds of that which passes the 100 mesh screen being fine enough to pass a 200 mesh screen.

9. A sulphur-coke composition containing approximately four parts of sulphur by weight and three parts of coke by weight,

from 25 to 75% by weight of the coke being fine enough to pass through a 100 mesh screen on which the balance remains and from 40 to 75% of that which passes the 100 mesh screen being fine enough to pass a 200 mesh screen. 15

In testimony whereof I affix my signature.

HARRY A. NOYES.